

March 17, 1959

G. H. WOOD, JR., ET AL

2,878,096

METHOD OF PRINTING ON WEB MATERIAL

Filed July 27, 1956

*Fig. 1.*



*Fig. 2.*



*Fig. 3.*



INVENTORS

George H. Wood, Jr.  
Charles Eric Neale  
Ralph E. Hawes

BY *Barlow & Barlow*  
ATTORNEYS.

# United States Patent Office

2,878,096

Patented Mar. 17, 1959

1

2,878,096

## METHOD OF PRINTING ON WEB MATERIAL

George H. Wood, Jr., East Greenwich, and Charles Eric Neale, Warwick, R. I., and Ralph Edson Hawes, New Bedford, Mass., assignors to The Apponaug Company, a corporation of Delaware

Application July 27, 1956, Serial No. 600,634

10 Claims. (Cl. 8—62)

This invention is a continuation in part of our application Ser. No. 498,916, filed April 4, 1955, now abandoned, and relates to printing with colors on woven web material.

Heretofore conventional textile roller printing even with the finest photoengraving techniques has not begun to duplicate on cloth the fine detail and continuous tone that is achieved on paper printed with shallow engravings such as roto or photogravure engravings. Attempts have been made to use with a photogravure engraved cylinder a printing paste having an emulsified aqueous solution of a dye or dye component with a water immiscible bodying composition but without commercial success.

To date there is only one successful method of duplicating on cloth the fine detail and continuous tone effects that are achieved on paper. This method involves a transfer print in which the pattern is firstly printed in all colors and complete detail on special paper on conventional paper printing equipment; then the whole pattern is transferred from the paper to the cloth by means of a suitable combination of heat, pressure and solvents. Fixation of the color on the cloth is then achieved by conventional means. This is a slow, laborious and costly process involving complex and expensive paper printing equipment, transfer equipment, paper, and the extraordinary precautions necessary when printing with inks in an inflammable all solvent system.

Our invention is a process whereby we can print directly on the cloth with conventional textile roller printing equipment, slightly modified, using roto- or photogravure engravings, and achieve the fine detail and continuous tone gradations of paper printing heretofore available only on cloth through the mechanism of the transfer print technique, thereby eliminating the necessity of paper printing equipment, paper, and the transfer operation.

Conventional textile roller printing equipment in essence has the characteristics that a web of cloth or the work is led through tension arrangements and laid on the surface of a fibre or fibre-rubber blanket known as a back grey or blanket which is being passed around an iron cylinder, the surface of which has been covered with several layers of heavy fabric known as lapping. The colors forming the pattern are applied to the cloth as it passes between the nips formed by the hand engraved cylinders as they rotate against the blanket. From thence the blanket or back grey is either washed and returned continuously or wound up separately while the cloth or work passes through or over a drying mechanism.

Conventional gravure paper printing equipment has the characteristics that a web of paper is led through tension devices, then through a nip formed by a rubber covered cylinder, and a roto- or photogravure engraved cylinder carrying one color in a portion of the pattern. From the nip, the paper web passes through a drying mechanism, then is returned to pass through a similar rubber covered cylinder-engraved cylinder nip where a second portion of the pattern is impressed on the paper surface followed by passage through or over a drying mechanism. The complete cycle of printing a portion of the pattern followed by drying may be repeated as many times as necessary to complete the pattern.

Our invention has the characteristics that a web of cloth

2

that has a smooth surface is led through tension devices and laid on the rubber covered surface of an iron cylinder. Colors and portions of the pattern are applied to the cloth as it passes through the nips formed by the roto- or photogravure engraved cylinders rotating against the covered surface. The cloth or work then passes through or over a conventional drying mechanism.

Paper, by its nature, has an inherent flatness and smoothness of surface that permits very fine printed detail to show on its surface. Conversely the usual cloth by its nature presents even in its finest form a relatively coarse and uneven surface and in most cloth constructions a much coarser and more uneven surface than paper. Consequently, the degree of printed detail possible on the usual cloth is limited conventionally by the coarseness of its surface.

Further, roller printing equipment for paper provides, in the form of a rubber covered cylinder, a very smooth even backing for the paper at the moment of color transfer from the engraved cylinder to the paper surface. Conversely, the roller printing for the usual cloth provides, in the form of a very coarse fabric lapping and surface textured fibre-rubber blanket or coarse fabric back grey, a relatively rough and uneven backing for the cloth at the moment of color transfer from the engraved cylinder to the cloth surface.

Consequently, the very fine detail roto- or photogravure engravings are not used for cloth printing because the fine detail is lost in the general coarseness of the cloth subjected to the printing operation.

It is customary in conventional textile roller printing to apply a relatively large amount of pressure to both extremities of the rollers, pressing them very tightly against the blanket and lapping. This is done to ensure the minimizing of any differences in color deposit on the surface of the cloth from edge to edge which might otherwise result because of the inherent coarseness of the cloth surface. However, this extreme pressure causes a distortion of the rollers, resulting in a bowing effect, there being less pressure on the center surface of the cloth than on the sides. To offset this unequal pressure and permit equal pressure to be exerted across the surface of the cloth, two steps are customarily taken:

The metal cylinder is made with a crowned or convex surface and/or the lapping is put on in such a way that it presents a crowned or convex surface over which the cloth passes.

The degree of crown or convexity of the backing for the cloth attempts to match the concavity of the surface of the rolls rotating against it under pressure. The result is under optimum conditions a curved nip exerting equal pressure at all points.

Gravure paper printing equipment, on the other hand, prints on a smooth surface (paper) and consequently does not require the extreme pressure to overcome inherent surface coarseness in order to provide an even color deposit from edge to edge of the paper. Thusly they naturally use a minimum of pressure on the engraved cylinder and of necessity provide an undistorted backing to the paper. The result is a straight nip through which the paper passes with equal though minimal pressure exerted at all points.

Our invention uses a cloth having a smooth flat surface. An example of such smoothness is that of a satin cloth, either as the cloth comes from the loom or is so formed smooth by calendering and thus does not require the curved conventional textile printing nip but allows the use of the delicate and more easily controlled straight type nip of the gravure paper printing technique.

Our invention does not depend on an emulsion type of printing paste. Rather many different types may be used and of less viscosity.

It is customary in conventional textile roller printing to directly gear drive the engraved cylinders which in turn because of the pressure with which they are forced against the lapping surface of the iron cylinder cause it to rotate at the same peripheral speed as that of the engraved cylinders. Contrarily, gravure paper printing equipment with an individual backing cylinder for each engraved cylinder, generally gear drives both backing and engraved cylinders. Our invention follows in this respect the textile printing principle, namely, driving the engraved cylinders and not the main large cylinder.

Reference may here be made to the drawing wherein Figure 1 is a diagrammatic view of the apparatus; Figure 2 is a similar view of a modified form; and Figure 3 is a similar view of a different modification.

The main large cylinder comprises an iron roll 10 with a heavy rubber covering 11 having a resiliency measuring 65 on the Plastometer scale and of good durability and then grinding it to the desired smoothness. The engraved rollers 12, 13, 14 apply the color and are driven and press against the rubber cover 11 sufficiently to drive this large roll. If a minimum amount of pressure of the engraved cylinders 12, 13, 14 against 11 is required, then a separate driver roller 15, as shown in Figure 2, of the same dimensions as the engraved cylinders 12, 13, 14 is pressed tightly against the surface 11 and gear driven at the same speed as 12, 13 and 14, which in turn causes the cylinder 10, 11 to rotate at the same peripheral speed as the rollers 12, 13, and 14. This is done when the pressure of the rollers 12, 13, 14 against 11 is insufficient to cause rotation of 10, 11 at the same speed as 12, 13, 14.

The first problem, that of surface flatness and smoothness without sizing or filling in printing finer detail on cloth than is customary, can be off-set by choosing a cloth of proper smoothness or by calendering the cloth to provide this. The degree of severity of calendering is dependent on the particular cloth construction but must be sufficient to impart a temporary smooth flat effect on the cloth surface. This provides a printing surface equally as smooth and even as satins. The smoothness is temporary, being completely removed during the operations subsequent to printing. No agents are present to make the smoothness in any way permanent. The only agents used to achieve the temporary smoothness are heat, pressure, and/or friction. Moisture may or may not be present in the cloth at the moment of calendering as desired for that particular construction of cloth.

In some fabrics such as rayon satins or some sateens, the cloth may be naturally smooth sufficiently to not require this calendering as is necessary for the usual cloth desired to be printed.

The second problem, that of providing for the flat, smooth, even cloth, a backing of relatively equal smoothness and evenness, can be solved in several ways, namely:

As shown in our drawing, by covering the iron cylinder against which the engraved rolls rotate with rubber 11 of the necessary resiliency (for example 65 on the Plastometer scale) and durability and grinding its surface to the required smoothness and evenness, we dispense with the blanket or back grey completely and run the smooth cloth between the series of nips formed by the rubber surface 11 of the iron cylinder and the engraved rolls.

Alternately, the iron cylinder surface could be covered with any natural or synthetic material which would have or be given the necessary surface smoothness and resiliency to allow the roto- or photogravure engraving to show on smooth, flat cloth.

Another form would be to use the surface of the iron cylinder 20 of Figure 3 as a smooth even backing, then passing a smooth faced fibre-rubber, plastic, or synthetic blanket 21 of the proper resiliency over the surface of the iron cylinder 20. The cloth 22 to be printed would pass on the outer surface of the blanket between nips formed by the blanket and the engraved cylinders 23, 24, 25 rotating against it.

Alternately, the iron cylinder surface 20 could be covered with any natural or synthetic substance that would provide in combination with the blanket used a support for the glazed cloth during printing of the required 5 smoothness, evenness, and resiliency.

Finally, a smooth surfaced natural or synthetic fibre back grey can be substituted for the blanket provided the covering of the iron cylinder in combination with the back grey gives a support for the cloth during printing 10 of the required smoothness, evenness, and resiliency.

The rollers which apply the printing material or paste are the tubular cylindrical shell textile printing type. The outer surface of one of these rollers, however, instead of being photoengraved as a textile roller conventionally is 15 with intaglio recesses to a depth of .003-.005 of an inch, which would cause smearing if used on the smooth surface cloth referred to above, is photographically engraved with an intaglio pattern having shallow recesses graduated from one micron to .0025 of an inch, usually not over .001 of an inch, to give continuous tone gradations 20 and provide perspectives as in photography. This process of engraving is usually referred to as gravure engraving, sometimes referred to as rotogravure or photogravure. The screen used for these rolls may be either a 150 or 25 175 line screen.

In preparing the material which is to be applied to the cloth and which gives the color to the cloth, we find some 30 are more easily wet with one solvent and others with a different solvent. For illustration, the vat dyestuff color paste consisting of the solid dyestuff in a water paste form is treated with an organic solvent, such for instance as mineral spirits or xylol, or any other solvent which will preferentially wet the dyestuff by enveloping it and, as it is insoluble in water, will thus separate it from the water. 35 The water is then removed by centrifuge or vacuum to leave the dyestuff mixed with the solvent. The dyestuff is then adjusted in the solvent so that there will be from 5% to 30% solids, 10% to 20% being that most usually used for the results required. This dyestuff paste is then 40 used in an amount by weight of 30%, while a printing vehicle consists of an emulsion of 70%. This printing vehicle emulsion comprises mineral spirits 30-70 parts, methylcellulose 2-10 parts, and water 68-20 parts. A satisfactory emulsion may be taken from these ranges of 45 mineral spirits 50 parts, methylcellulose 3 parts, and water 47 parts.

By adding the dyestuff in the solvent to this emulsion, we obtain the pigment of the vat dye color in an oil phase 50 so that it becomes wet with oil instead of wet with water and thus in a water in oil emulsion, which we prefer. The vat color could be wet with oil and in an oil in water emulsion. Water in the discontinuous phase serves to thicken the emulsion.

Viscosity is measured in terms of centipoise according 55 to the Saybolt viscometer. The usual printing paste for conventional photoengraved rollers has a viscosity of from 6000 to 8000 centipoises, which is much thicker than the printing paste which we use for the fine engraving of this invention. Our paste is in the order of from 200 to 3000 centipoises, which is much thinner than heretofore ever used on cloth.

In some cases the pigment dissolved as heretofore mentioned may be added directly to a printing vehicle consisting of phenol formaldehyde resin which might be modified by rosin and which is known as "Amberols" together 60 with soaps such as triethanolamine stearate or diethanolamine stearate.

Although we have referred to vat colors, other colors may be used according to the material to be printed, for 65 example, pigment colors, acid colors, acetate or dispersed colors, basic colors, sulfur colors, azo colors, or direct colors. Acetate colors for fibers of nylon, acetate, polyester, acrylic, etc., are used wet with oil, in a water in oil system or wet with water, in an oil in water system.

70 In the case of direct colors we use the colors wet with or

dissolved in water, in a water in oil or oil in water emulsion.

A fabric which is printed with vat colors in this manner is permitted to dry and is then padded in the usual padder with caustic soda and sodium hydrosulphite. The caustic soda is used in a quantity dry of from 2-12 ounces and the sodium hydrosulphite is used in the same amount of 2-12 ounces each per gallon of water. It is usual that these two be used in equal amounts, although one may be used in a greater amount than the other. The quantities given are variable depending upon ease or difficulty of the reduction of the particular color which may be used. Some colors require a greater amount than others.

After padding with the mixture above, the web of material is passed through a steam chamber at a speed so it will remain in the steam chamber from 5-30 seconds. Usually 10-20 seconds is suitable for the results desired. This steam treatment is followed by the usual oxidation and soaping process of Vat prints after ageing.

The above may be used for printing colors on fabrics of different materials, such as fibers of silk, cotton, wool, rayon, acetate, nylon, acrylic or polyester or mixtures of any of these.

Reproduction of detail is a function of fineness of screen, shallowness of engraving and smoothness of surface being printed.

Maximum detail requires the finest of screens (150-175 lines per inch) with shallow etch engraving (less than .001" depth) and strong color (10-15% dyestuff on solids basis for vat colors). The print color must be in either (1) an all solvent system or (2) a water in oil emulsion. An all water system or an oil in water emulsion will not give maximum detail. The viscosity of the print color should be less than 1500 centipoises as measured with a Brookfield viscometer for maximum detail. A 150-175 line screen etched to .001" depth will not print out on any fabric in complete detail without calendering the surface of the cloth before printing.

An 85-100 line screen etched to .002" maximum depth will print on the flat surface of the normal flat woven fabric but to get the maximum color value it is necessary to use the vat color in pigment form (not mixed with the chemicals normally used in vat color printing) and develop the color by the flash ageing technique described herein under Example 2. This engraving will not give detail on textured surface fabrics without calendering.

The print color could be made up in an all solvent system—a water in oil emulsion—an oil in water emulsion or an all water system.

The viscosity of the print color should be from 1500-2500 cps. (centipoises).

In patterns with overlays (one color falling on another wet on the cloth) it is preferable to use an all solvent or water in oil printing vehicle to avoid marking off. By this method the first color printed is rapidly absorbed by the cloth and the next color falling on the first will be absorbed slower but not slow enough to cause marking off or spreading of the color. In conventional printing with colors made up with starches and gums, patterns with overlays cause considerable trouble due to the double layer of color which is not absorbed by the cloth fast enough to prevent marking off and spreading out beyond the printed area before or during the drying process.

Gravure screens of 65 lines etched to .003" or greater depth can be used with conventional colors and printing equipment on the ordinary flat surface fabric without calendering. Textured surface fabrics would require calendering to reproduce the pattern properly. The depth of shade is limited to the amount of chemicals that could be carried in the vehicle for development of the color. Using conventional colors by this method it is not possible to get the deep shades that could be obtained by use of finer screens and more shallow etching with all solvent or water in oil printing colors as described above.

This engraving could be printed with the vat color in

pigment form in an all solvent system; water in oil or oil in water emulsion or in an all water system and the color developed by flash ageing.

The viscosity of the colors would be above 2500 centipoises.

*Examples of printing by the described methods*

I. Cotton cloth of 80/80 construction 4.00 yards per pound weight is bleached as for conventional printing, 10 then is further prepared for our invention by being passed through a nip of a conventional rolling calender at speed of 20 yards per minute, a pressure of 1½ tons per linear inch of calender nip, and a temperature of 300° F. so that the cloth surface becomes very markedly, though non-permanently, flattened to the extent of being of similar smoothness and evenness as the average satin surface; the cloth then being passed through the modified printing machine as previously explained, the design being printed on from the rotogravure or photogravure engraved rollers 15 by colors made as in the following illustration:

5 parts of a natural gum are dissolved by boiling in

30 parts of water, then

30 parts of a 50% potash solution and

5 parts of glycerine are added to the hot gum solution.

Cooling is started and

10 parts of sodium formaldehyde sulfoxylate are added.

Agitation is continuous and slow throughout the mixing until the paste is cool. At this time the addition is made of 20 parts of commercial Anthraquinone Vat Orange RRT paste, Color Index #1098.

The paste will be water paste of about 600 centipoises viscosity.

Any of the commercially available Vat color pastes 35 sold for conventional textile printing can be substituted for the Vat Orange RRT.

After printing with our invention, the cloth is passed over steam heated drying cylinders of conventional design, passed through a relatively air-free, saturated steam atmosphereager of conventional design operating at an interval temperature of 212° F. to 235° F. for a period of from 4-20 minutes followed by immersion in and passage through conventional oxidizing and soaping baths.

II. Cloth preparation, printing, and drying as in Example #1.

The alkyd resin herein referred to may be prepared by reacting

140 parts, by weight, of glycerol,

200 parts phthalic anhydride and

230 parts linseed oil fatty acids.

at 230° centigrade to give an acid number of less than 9. The alkyd resin might be made by reacting

55 220 parts glycerol

300 parts phthalic anhydride and

250 parts castor oil fatty acids.

at 230° centigrade until the acid number is 8. The resin thus produced should then be reduced with equal parts of a solvent; such as xylol or toluol or a hydrogenated petroleum naptha with an evaporation end point of less than 200° centigrade. Any of these solvents could be replaced by pine oil or the various solvents could be mixed.

The alkyd resin could likewise be modified with soya oil or other oils and the acid number might be from 5 to 9. We have found the Glyptal 91033 (a General Electric Company product) to be suitable and also Aridye Clear 6214. Also Glyptal 2503, 2520, 2480, and 2477. Glyptal 2520 is a castor oil modified alkyd with an acid number of 4-5; 2503 is a soya oil alkyd with an acid number of 30-35; 2480 is a castor oil alkyd with an acid number of 4-5—somewhat similar to 2520 but giving emulsion of less viscosity and not as stable; 2477 is a castor oil alkyd with higher oil content (45%) than

2520 and 2480 (25%) and an acid number of 4-6 giving a softer film than 2520 and 2480. It is very suitable for our process because of its lubricating character.

Print color formulated as a water in oil emulsion as follows:

3 parts of a clear solvent solution of an alkyd resin prepared as above are stirred into

8 parts of a mixture of aliphatic naphtha in the distillation range of 300° F. to 400° F. Amsco #46 (American Mineral Spirits) to form the oil phase.

20 parts of Anthraquinone Vat Brilliant Violet 4RN Color Index #1104 in a flushed form is stirred into the above to form the color-carrying oil phase.

69 parts of cold water are then slowly added with high speed mixing to the above to form the stable water in oil emulsion of about 1900 centipoises viscosity suitable for printing with our invention.

After drying, the cloth is passed through a short bath containing as ingredients

6 oz. caustic soda, and  
6 oz. sodium hydrosulphite

1 gallon water

squeezed by a set of rubber rollers to retain 80% of its own weight in wet pickup from the bath, passed quickly into a relatively air-free saturated-steam atmosphere ager operating at a temperature of 214° F. to 280° F. for a period of time of from 5 to 60 seconds, then into and through conventional oxidizing and soaping baths. This technique of Vat color fixation is conventionally known as Flash Ageing and is described in U. S. Patent #2,587,905.

Vat colors are manufactured and marketed to the textile trade as pigments dispersed in and wet by water. However, they have been transferred by some manufacturers from their conventional water dispersed state to a solvent or oil dispersed state by techniques common to the pigment trade and known as Flushing for use as inert pigments in paints or occasionally in textile pigment printing applications.

We find that carrying the Vat color pigment in the oil phase of a water in oil emulsion or oil in water emulsion and fixing on the cloth by the Flash Ageing technique provides us with a printing color paste or ink that allows full reproduction of any conventional Roto or photogravure engraving when used in printing with our invention.

All commercially available Vat color pigments that can be flushed are applicable as in this illustration.

III. Cloth preparation, printing, drying, Flash Ageing, oxidizing, and Soaping are as in Example II. Color ink make-up as follows:

1½ parts of sodium alginate Keltex (The Kelco Company) are dissolved with agitation in

78½ parts of water to form the water phase

20 parts of Anthraquinone Vat Brilliant Violet 4RN,

Color Index #1104 in the flushed form are then added slowly to the water phase with high speed mixing to form a stable oil in water emulsion of about 1600 centipoises viscosity suitable for printing with our invention.

N. B.—The various resins or bodying agents added to the Flushed Vat color either to aid in the flushing process or to provide a smooth commercially workable color paste generally act as emulsifying agents. When they are absent or are not sufficient to give a practical emulsion, the addition of 3-5 parts of diethanolamine-stearic acid condensate Bradsyn APP (Bradford Soap Works) to the oil phase creates a satisfactory emulsion.

IV. Cloth, preparation, printing, and drying are as in Example II.

Color ink make-up as follows:

3 parts of an alkyd resin as in Example II are stirred into 20 parts of aliphatic naphtha in the distillation range of 300° F. to 400° F. Amsco #46 (American Mineral Spirits) to form the oil phase.

5 3 parts of Pontamine Fast Yellow NNL conc. 175%, Color Index #814 (E. I. du Pont de Nemours & Co.) and

10 parts of urea are dissolved by boiling in 64 parts of water to form the water phase.

10 The water phase is then cooled and filtered, then added slowly under high speed mixing to the oil phase to form the complete water in oil emulsion of about 1450 centipoises viscosity suitable for printing with our invention. After printing and drying, the cloth is aged or steamed as usual for the fixation of direct colors. It is then given the customary washing.

V. Cloth, preparation, printing, drying, Flash Ageing, oxidizing, and Soaping are as in Example II.

Color ink make-up as follows:

10 parts of an emulsifying agent such as Bradsyn APP (Bradford Soap Works) referred to above, are melted into

20 parts of aliphatic naphtha in the dilution range of 300° F. to 400° F. Amsco #46 (American Mineral Spirits) to form the oil phase.

1 part of sodium alginate Keltex (Kelco Co.) is dissolved in

48 parts of water, then

20 parts of Anthraquinone Vat Blue GCD, Color Index #1112 in the commercial water dispersed paste form are added to make the water phase.

The oil phase is added slowly to the water phase under high speed mixing to form a stable oil in water emulsion of about 475 centipoises viscosity suitable for printing with our invention.

VI. Cloth, preparation, printing, drying, Flash Ageing, oxidizing, and Soaping are as in Example II.

Color ink make-up as follows:

3 parts of vat color Ponsol Golden Orange RRTK powder, Color Index #1098 are ball milled into

37 parts of xylol

20 parts of a phenol-formaldehyde resin such as Amberol ST 137 (Rohm and Haas) and

45 10 parts of a solvent soluble soap such as Bradsyn APP (Bradford Soap Works) are dissolved by heat and agitation in

30 parts of xylol

50 The xylol containing the Orange RRTK is then added to the xylol containing the resin and soap to give an all solvent type ink of about 1275 centipoises viscosity suitable for printing with our invention.

VII. Example of a Direct Color on Rayon

A viscose rayon fabric previously calendered to give the required degree of smoothness of surface may be printed with a direct color made up as the following example.

60 8 parts of Direct Blue 86 Color Index No. 74180 are pasted with

4 parts of ethylene glycol mono ethyl ether cellosolve (Carbide and Carbon Chemical Co.) then mixed with

20 parts of boiling water in which

20 parts of urea has been previously dissolved.

1 part of trisodium phosphate is then dissolved in the above mix.

47 47 parts of a gum Karaya solution of such strength as to give a final viscosity of 500 centipoises is then added to give

100 parts total of color paste ready to print.

After printing and drying, the cloth is steamed 8-10 minutes to fix the color and is then washed and finished as usual for this cloth.

**VIII. Example of a Pigment Color on Cotton**

A cotton fabric prepared for printing by calendering to give the required degree of surface smoothness may be printed with Pigment colors made up according to the following example

25 parts of a paste composed of

20 parts Indanthrene Blue CE C. I. 1112

2 parts ethyl cellulose

78 parts solvent mixture of

50 parts xylol, 5 parts pine oil, 45 parts mineral spirits (aromatic petroleum distillate)

75 parts of a mixture composed of

15 parts ethyl cellulose

85 parts solvent mixture

(50 parts xylol, 15 parts pine oil, 10 parts methanol, 25 parts mineral spirits (aromatic petroleum distillate))

The ethyl cellulose can be of a type to give a viscosity of approximately 500 centipoises in the finished color or the viscosity can be controlled to approximately 500 by varying the amount of ethyl cellulose solution added and making up to 100 with solvent.

After printing, the cloth is dried, cured at 280° F. five minutes, and then washed and finished in the usual manner.

**IX. Example of a Sulphur Color on Cotton**

A cotton fabric which has been calendered to give the required smooth surface may be printed with a sulphur color prepared as follows:

35 parts of So-Dye-Co Printing Green SP Paste (Southern Dyestuff Co.) is mixed with

65 parts of a gum Karaya solution of such strength as to give a final viscosity of 500 centipoises to give

100 parts total of color paste ready to print.

After printing and drying, the cloth is padded through a solution of 4 oz. per gal. sodium hydrosulphite and 4 oz. per gal. caustic soda and, while still wet, steamed at 220-280° F. for 10-30 seconds, then washed, soaped, and finished as usual.

**X. Example of an Acid color printed on silk previously prepared to the required degree of surface smoothness**

10 parts of Acid Blue 83 Color Index No. 42660 are pasted with

5 parts of resorcin, then further mixed with

30 parts of hot water in which

10 parts of urea and

2 parts of ammonia water 28% has been previously dissolved.

43 parts of a gum Karaya solution of such strength as to give a final viscosity of 500 centipoises is then added to give

100 parts total of color paste ready to print.

After the printing and drying, the silk is steamed for 8 to 10 minutes in a Mather Platt ager and is then washed and finished as usual for the cloth.

**XI. Example of a Dispersed Color on Acetate**

An Acetate fabric previously prepared to the required degree of smoothness may be printed with dispersed color made up as follows:

10 parts of Disperse Blue 1 Color Index No. 64500 are pasted with

10 parts of hot water, then further mixed with

15 parts of boiling water in which

5 parts of urea have been previously dissolved

50 parts of a gum Karaya solution of such strength as to give a final viscosity of 500 centipoises is then added to give

100 parts total of color paste ready to print.

After the printing, the cloth is dried, steamed for 8 to 10 minutes, washed, and finished in the usual manner.

The following grouping of examples may also be made. The method of make-up for all may be any one of the following:

- (1) Oil in water emulsion-color in oil
- (2) Oil in water emulsion-color in water
- (3) Water in oil emulsion-color in oil
- (4) Water in oil emulsion-color in water
- (5) All water-color in water
- (6) All solvent-color in solvent

|    | Color     | Method of Fixing                                                                                           | Fiber printed on—                                                                                                                                                                            |
|----|-----------|------------------------------------------------------------------------------------------------------------|----------------------------------------------------------------------------------------------------------------------------------------------------------------------------------------------|
| 15 | Pigment   | (a) Thermoplastic resins and/or<br>(b) Thermosetting resins                                                | All fibers.                                                                                                                                                                                  |
| 20 | Vat       | (a) Alkaline reduction and Steam.<br>(b) Acid Reduction and Steam.<br>(c) Solid solution                   | Cotton, Silk, Wool, regenerated cellulose (Bemberg, Viscose), cellulose diacetate (Acetate), cellulose triacetate (Arnel), acrylic (Orlon), polyester (Dacron).                              |
| 25 | Sulphur   | Alkaline reduction and Steam.                                                                              | Cotton, Silk, Wool, regenerated cellulose (Bemberg, Viscose).                                                                                                                                |
| 30 | Direct    | (a) Steam with or without overpadding or addition of extra chemicals in print paste.<br>(b) Solid solution | Cotton, Silk, Wool, Nylon, regenerated cellulose (Bemberg, Viscose), cellulose diacetate (Acetate), acrylic (Orlon), polyester (Dacron), polyacrylic (Acrlan), cellulose triacetate (Arnel). |
| 35 | Acid      | Above as for Direct                                                                                        | Cotton, Silk, Wool, Nylon, regenerated cellulose (Bemberg, Viscose), cellulose diacetate (Acetate), acrylic (Orlon), polyester (Dacron).                                                     |
| 40 | Dispersed | Solid solution with or without carrier                                                                     | Nylon, cellulose diacetate (Acetate), acrylic (Orlon), polyester (Dacron).                                                                                                                   |

35 For each fabric there is a range of temperatures, pressures, and speeds of calendering to achieve the requisite flatness and evenness of surface for printing with our invention that depends on construction and on fiber used. (E. g. the thermoplastic synthetic fibers can naturally not be subjected to temperatures that will melt them.)

40 Additionally, for each fabric and fiber there are applicable groups of colors, but each commercially available color can be introduced into one or more of the ink examples with only minor or no modification of ink make-up procedure, printed by our invention on the cloth on which it is normally conventionally used and fixed by conventional means.

We claim:

1. In the process of printing, providing a single ply 50 of woven cloth, calendering the cloth with sufficient pressure to provide a non-permanent smooth surface and thereafter printing by continuously rolling in direct contact with said smooth surface a cylindrical surface having an intaglio engraved photogravure reproduced pattern 55 of a depth of from one micron to .003 of an inch carrying in its depressions a printing paste of from 200 to 3000 centipoises viscosity.

2. In the process of claim 1 wherein the cloth is backed up by a rotating resilient surface.

60 3. The process claimed in claim 1, wherein the backing comprises a resilient surface which is modified by a smooth surfaced synthetic film to collect and remove excess printing material.

4. In the process of claim 1 wherein the calendering 65 is done in the absence of a filling in the cloth.

5. The process claimed in claim 1, wherein the printing 70 surface is etched with a 150-175 line screen to a depth less than .001, the printing paste has a viscosity of less than 1500 centipoises and is formed by a strong color carried in an all-solvent system or a water-in-oil emulsion.

6. In the process of claim 1 wherein the printing paste 75 is an emulsion of water and oil and the color comprises 20% of a 5-30% vat color in flushed form and a 1-6% alkyd resin, 5-30% mineral spirits, and the balance to 100% water.

7. In the process of claim 1 wherein the printing paste is an emulsion of water and oil and the color comprises 30% of a 5-30% solid vat color pigment and printing vehicles 70% comprising mineral spirits 30-70, methylcellulose 2-10, water 68-20 parts by weight.

8. In the process of claim 1 wherein the printing paste is an emulsion of water and oil and the color is a vat color in the oil phase and fixation of the color is had after printing.

9. In the process of claim 8 wherein the fixation is by padding with sodium hydroxide 2 to 12 ounces sodium hydrosulfite 2 to 12 ounces per gallon of water.

10. The process of claim 8 followed before drying by ageing.

## References Cited in the file of this patent

## UNITED STATES PATENTS

|           |             |               |
|-----------|-------------|---------------|
| 454,854   | Cochran     | June 30, 1891 |
| 1,135,043 | Neuberger   | Apr. 13, 1915 |
| 2,175,051 | Bromley     | Oct. 3, 1939  |
| 2,202,283 | Cassel      | May 28, 1940  |
| 2,264,475 | Learnard    | Dec. 2, 1941  |
| 2,288,992 | Cassel      | July 7, 1942  |
| 2,361,454 | Cassel      | Oct. 31, 1944 |
| 2,370,461 | Heberlein   | Feb. 27, 1945 |
| 2,587,905 | Saville     | Mar. 4, 1952  |
| 2,594,899 | Fordemwalt  | Apr. 29, 1952 |
| 2,597,281 | Borstelmann | May 20, 1952  |